

## 1

3,128,204

## PROCESS OF PREPARING PHOTOCODUCTIVE LAYERS FOR ELECTROPHOTOGRAPHY

Gustav Schaum and Hildegard Haydn, Leverkusen, Germany, assignors to Agfa Aktiengesellschaft, Leverkusen, Germany, a corporation of Germany

No Drawing. Filed Nov. 13, 1957, Ser. No. 696,024

Claims priority, application Germany Nov. 14, 1956

5 Claims. (Cl. 117—221)

The present invention relates to photoconductive layers for electrophotography.

For the production of photoconductive layers for electrophotography it is known to use certain inorganic or organic photoconductive compounds. Examples of such compounds are sulfur and selenium; oxides, sulfides and selenides of zinc, cadmium, mercury, antimony, bismuth, and lead, and also anthracene and anthraquinone. These substances are applied to an electrophotographic plate, especially a plate consisting of metal or another material, for example paper, or to a sheet or foil produced from a film-forming plastic. If necessary, the photoconductive substance can be held dispersed in an electrically isolating layer-forming binder. Such layers are produced by means of coating solutions in which the binders are either dissolved or dispersed and in which the electroconductive substances are dispersed. Such photoconductive layers are disclosed, for instance, in United States Patents Nos. 2,297,691; 2,357,809; 2,727,807; 2,727,808; 2,735,784; and 2,735,785, and in French Patents Nos. 1,113,933; 1,122,275; 1,125,235; and 1,136,146.

The photoconductive layers which are produced from aqueous coating solutions in which the binders are dispersed suffer from the disadvantage that they readily take up moisture from the air owing to the presence of wetting agents and salts, so that the conductivity of the layer in the dark is often raised to such a degree that its image reproduction characteristics are impaired.

It has now been found that the dark conductivity of the photoconductive layers can be reduced substantially if waterproofing agents are added to the dispersions. These waterproofing agents can be of various types.

Suitable waterproofing agents are the following:

(a) paraffin wax or similar high-molecular hydrocarbons which are preferably applied in the form of their aqueous emulsions; such emulsions are, for instance, disclosed in British Patents Nos. 477,830; 492,742; 469,642, and 627,356.

(b) Complex compounds of the Werner type in which a trivalent nuclear chromium atom is coordinated with an acyclic carboxylic acid (alkylcarboxy) group having at least ten carbon atoms, as they are disclosed in United States Patent No. 2,273,040. A suitable compound is for instance chromium stearoyl chloride.

(c) Fatty acids salts of polyvalent metals, more especially, fatty acids salts of aluminum, titanium, zirconium, and chromium.

(d) Metal compounds which are capable of hardening gelatin or other proteins, such as zirconium oxychloride, phosphotungstic acid, chrome alum, chromium acetate, chromic acid, alum, and cerous nitrate.

The water-repellent or waterproofing agents are preferably applied in the following quantities:

The paraffin emulsions when used as 10% emulsions in

## 2

amounts of 20–120%, the compounds quoted under (b) and (c) in amounts of 3–30%, and the compounds disclosed under (d) in amounts of 0.01–1% as calculated on the binding agent.

As film-forming agents for the photoconductive layers in which the photoconductive substances are dispersed there may be used natural or synthetic resins or resinoids preferably such as are soluble in organic solvents, these film-forming agents being used in form of aqueous dispersions as disclosed, for instance, in French Patent No. 1,136,146. After coating, the layers produced from said dispersions may be subjected to a final condensation or final polymerization by heat treatment at temperatures of about 80–150° C. for about 2 to 30 minutes after being dried. Aqueous dispersions of polymeric substances which are soluble in organic solvents, such as melamine-formaldehyde or urea-formaldehyde resins, xylene-formaldehyde resins, polymers based on vinyl chloride, vinylidene chloride, vinyl ethers, acrylic esters, methacrylic esters, acrylic amides, such, for example, as methacrylic amide, aromatic vinyl compounds, such, for example, as styrene, isoolefins, such, for example, as isobutylene, copolymers based on the aforementioned compounds, such, for example, as copolymers of vinyl chloride and butyl acrylate, vinylidene chloride and butyl acrylate, synthetic elastomers, such, for example, as copolymers of butadiene and styrene, butadiene and acrylonitrile, and also copolymers of dienes with a preponderant proportion of styrene and/or acrylonitrile or other vinyl compounds, as well as polyamides, polyurethanes, polyesters of polycarboxylic acids and polyhydric alcohols, polycarbonates, cellulose esters, rubber and the like, are, for example, employed.

For the production of the photoconductive layers there may be used photoconductive inorganic or organic substances, for example sulfur and selenium; oxides, sulfides, selenides and iodides of cadmium, mercury, antimony, bismuth, thallium, molybdenum, aluminum, lead or zinc; arsenic trisulphide; cadmium arsenide; lead chloride; anthracene; benzidine; anthraquinone; acenaphthene; fluoranthene; naphthalene; chrysene; quinone; gallic acid; and microcrystalline paraffin wax. Terphenyl or p-di-phenyl benzene, benzanthrone, 1,5-dicyanonaphthalene, 1,4-dicyanonaphthalene, aminophthalonitrile and nitrophthalonitrile are also particularly suitable.

The coating solution which is used for the production of the photoconductive layers comprises at least one of the aforementioned substances and a film-forming binding agent, the electric specific resistance of which must be higher than that of the photoconductive substance and preferably also higher than that of the layer support. The best results are obtained with binding agents the electric specific resistance of which amounts to at least  $10^{10}$  ohms per centimeter.

The quantitative ratios between the photoconductive substances and the binding agents may vary within wide limits. It is preferred to apply the photoconductive substance in amounts of 1 part per 0.3–2 parts by weight of binding agent, and in amounts of 5–60 grams per square meter of photoconductive layer.

As a support for the photoconductive layer there may be used paper or metal plates, such as zinc, aluminum, or brass plates. Furthermore, thin foils of cellulose hydrate, cellulose esters or of polyamide come into question.

The processing of the disclosed materials is carried out in the usual manner. The materials are first made sensitive to light by giving them an electrostatic charge on the coating side in the dark, for instance, by means of a corona discharge. The material is then exposed by any of the conventional photographic procedures. The latent image obtained is developed by applying a pigmented resin powder carrying an electrostatic charge which is opposite to that of the photoconductive layer.

*Example 1*

120 cc. of a 30% aqueous dispersion of a heat-hardenable melamine-formaldehyde resin,  
110 cc. of water, and  
40 g. of zinc oxide

are thoroughly mixed in a ball mill and 1 cc. of a 3% zirconium oxychloride solution is added. The dispersion is cast on a paper or metal support and dried. This dispersion is not stable for very long, because condensation proceeds very rapidly. The dispersion must therefore rapidly be cast after adding the zirconium oxychloride.

*Example 2*

120 cc. of a 30% aqueous dispersion of a melamine-formaldehyde resin as described in Example 1,  
110 cc. of water  
40 g. of zinc oxide, and  
30 g. of a 10% aqueous paraffin wax emulsion  
are thoroughly mixed in a ball mill, cast onto a support in the usual manner and dried. The paraffin wax emulsion can also be added just before casting.

*Example 3*

100 cc. of a 30% aqueous dispersion of a melamine-formaldehyde resin as described in Example 1,  
90 cc. of water,  
60 g. of zinc oxide,  
20 cc. of a 10% paraffin wax emulsion, and  
7 cc. of 30% formalin

are treated as above, it being advisable to add the formalin just prior to casting. Instead of formalin, a corresponding quantity of zirconium oxychloride or phosphotungstic acid may be added to the mixture.

In the foregoing examples there may be used instead of the melamine-formaldehyde resin a urea-formaldehyde resin which is heat hardenable.

*Example 4*

40 g. of zinc oxide are added to 50 cc. of a 35% aqueous emulsion of a copolymer of butadiene-acrylonitrile and styrene (40:40:20) after addition of 80 cc. of water. To this dispersion there are added 1.5 g. of chromium stearoyl chloride. After treating the dispersion for 2 hours in a ball mill, it is coated on a paper support and dried at 70° C.

*Example 5*

40 g. of zinc oxide are added to 100 cc. of a 35% aqueous dispersion of a copolymer of vinyl chloride, and acrylic acid and ethyl acrylate. To this dispersion there are added 25 cc. of an aqueous 10% paraffin wax emulsion. After treating in a ball mill for 2 hours, 100 cc. of water and 10 cc. of ammonia are added. Thereafter the dispersion is cast onto a paper support and dried at 80° C.

What we claim is:

1. A process of producing an electrophotographic plate which comprises mixing together in a ball mill zinc oxide, an aqueous dispersion of a heat-hardenable melamine-formaldehyde film-forming resinous binding agent in an amount between 0.3 and 2 parts by weight of the resin per part by weight of the zinc oxide, and an aqueous emulsion of paraffin wax in an amount between 2 and 12 percent by weight of the resinous binding agent based on

5 the paraffin wax content of the emulsion, and subsequently applying the said aqueous dispersion to a conductive support in such amount that the photoconducting insulating layer deposited therefrom contains between 5 and 60 grams of zinc oxide per square meter, and subsequently drying the said coated conductive support.

2. A process as defined in claim 1 in which the aqueous dispersion with which the conductive support is coated contains the following ingredients in proportions represented by the following quantities:

- (i) 40 grams of zinc oxide,
- (ii) 120 cubic centimeters of an aqueous dispersion of a heat-hardenable melamine-formaldehyde resin containing 30 percent by weight of resin,
- (iii) 110 cubic centimeters of water, and
- (iv) 30 grams of an aqueous emulsion of paraffin wax containing 10 percent by weight of paraffin wax.

3. A process of producing an electrophotographic plate which comprises mixing together in a ball mill zinc oxide, an aqueous dispersion of a heat-hardenable melamine-formaldehyde film-forming resinous binding agent in an amount between 0.3 and 2 parts of the resin per part of the zinc oxide, together with a waterproofing substance of the group consisting of

- (i) an aqueous emulsion of paraffin wax in an amount between 2 and 12 percent by weight of the resinous binding agent based on the paraffin wax content of the emulsion, and
- (ii) zirconium oxychloride in an amount between 0.1 and 1 percent by weight of the resinous binding agent,

and subsequently applying the said aqueous dispersion to a conductive support in such amount that the photoconducting layer deposited therefrom contains between 5 and 60 grams of zinc oxide per square meter, and subsequently drying the said coated conductive support.

4. A process as defined in claim 3 in which the aqueous dispersion with which the conductive support is coated contains the following ingredients in proportions represented by the following quantities:

- (i) 40 grams of zinc oxide,
- (ii) 120 cubic centimeters of an aqueous dispersion of a heat-hardenable melamine-formaldehyde resin containing 30 percent by weight of resin,
- (iii) 110 cubic centimeters of water, and
- (iv) 1 cubic centimeter of an aqueous solution of zirconium oxychloride containing 3 percent by weight of zirconium oxychloride.

5. A process as defined in claim 3 in which the aqueous dispersion with which the conductive support is coated contains the following ingredients in proportions represented by the following quantities:

- (i) 60 grams of zinc oxide,
- (ii) 100 cubic centimeters of an aqueous dispersion of a heat-hardenable melamine-formaldehyde resin containing 30 percent by weight of resin,
- (iii) 90 cubic centimeters of water,
- (iv) 20 cubic centimeters of an aqueous emulsion of paraffin wax containing 10 percent by weight of paraffin wax, and
- (v) 7 cubic centimeters of a 30 percent aqueous solution of formaldehyde.

References Cited in the file of this patent

UNITED STATES PATENTS

|           |               |               |
|-----------|---------------|---------------|
| 2,273,040 | Iler          | Feb. 17, 1942 |
| 2,287,348 | Hayden        | June 23, 1942 |
| 2,391,621 | Powell et al. | Dec. 25, 1945 |
| 2,394,009 | Pollard       | Feb. 5, 1946  |
| 2,399,489 | Landes        | Apr. 30, 1946 |
| 2,663,636 | Middleton     | Dec. 27, 1953 |
| 2,748,095 | Kling         | May 29, 1956  |
| 2,875,054 | Griggs et al. | Feb. 24, 1959 |

(Other references on following page)

## UNITED STATES PATENTS

2,901,348 Dessauer et al. ----- Aug. 25, 1959  
 2,959,481 Kaucera ----- Nov. 8, 1960  
 2,990,279 Crumley et al. ----- June 27, 1961  
 2,993,787 Sugarmann ----- July 25, 1961  
 2,997,387 Tanenbaum ----- Aug. 22, 1961

## FOREIGN PATENTS

543,624 Belgium ----- Dec. 30, 1955  
 201,301 Australia ----- May 19, 1956  
 1,136,146 France ----- May 9, 1957

## OTHER REFERENCES

Wainer: Photographic Engineering, vol. 3, No. 1, pp. 12-22 (1952).  
 5 Young et al.: R.C.A. Review, vol. XV., No. 4, pp. 469-484, December 1954.  
 Mees: The Theory of the Photographic Process, Macmillan (1954), pp. 73-84.  
 Webster's New International Dictionary, 2nd Ed. 10 (1954), p. 1771, "paraffin."